

Feb. 15, 1949.

J. B. DUKE

2,461,813

CONCENTRATION OF PHOSPHATE MINERALS

Filed Nov. 14, 1945



INVENTOR  
JAMES B. DUKE  
BY

Williams, Rich & Moore  
ATTORNEYS

## UNITED STATES PATENT OFFICE

2,461,813

CONCENTRATION OF PHOSPHATE  
MINERALS

James B. Duke, Lakeland, Fla., assignor to Minerals Separation North American Corporation, New York, N. Y., a corporation of Maryland

Application November 14, 1945, Serial No. 628,585

7 Claims. (Cl. 209—166)

1

The present invention relates to concentration of phosphate minerals from their ores, and may be regarded as an improvement upon the method covered by the patent to Arthur Crago No. 2,293,640, issued August 18, 1942, now owned by the assignee of the present application.

That Crago patent describes and claims a method of concentrating phosphate minerals from their ores, which comprises subjecting the ore in an aqueous pulp to a concentrating operation with reagents to separate a rougher concentrate of the phosphate values admixed with entrained siliceous gangue, treating the rougher concentrate with a mineral acid to remove the effect of the reagents used in its production, and thereafter subjecting the rougher concentrate in an aqueous pulp to a concentrating operation to separate a collected material largely composed of the entrained siliceous gangue, thereby producing a final phosphate concentrate.

The reagents, described in the Crago patent as useful in the first step of that method, are such negative-ion agents as the higher fatty acids, such as fish-oil fatty acid and oleic acid and their soaps, the resin acids and their soaps, wood by-products fatty acids, naphthenic acids and their salts, the higher sulpho-fatty acids and their salts with the proper bases, the acid esters of high-molecular-weight aliphatic alcohols with inorganic acids and their alkali-metal and alkaline-earth-metal salts, the higher xanthates, etc. The reagents described as useful in the last step of that method are of the positive-ion type such as the higher aliphatic amines and their salts with water-soluble acids, the esters of amino-alcohols with high-molecular-weight fatty acids and their salts with water-soluble acids, the higher alkyl-O-substituted isoureas and their salts with water-soluble acids, the resin amines and their salts with water-soluble acids, the higher aliphatic quaternary ammonium bases and their salts with water-soluble acids, the higher alkyl pyridinium salts of water-soluble acids, the higher alkyl quinolinium salts of water-soluble acids, etc. It is also stated in that patent that the use of an anionic active fatty acid compound is preferred in the carrying out of the first concentrating operation, while the use of a cationic-active amine compound is preferred in the carrying out of the second concentrating operation. In performing the intermediate step between the two concentrating operations, the mineral acid employed is described in that patent as preferably sulfuric acid because of its low cost. These various re-

2

agents are useful in the improved method of the present invention.

The Crago patent also states that in the carrying out of the concentrating operations used in practicing the method of that patent, any concentrating device may be used which is capable of discharging the collected material in such forms as floating froth, skin or surface float, individual agglomerates, etc.; and that such devices include flotation machines and gravity-concentrating tables, the collected material being discharged in the case of the former in the form of a floating froth over the lip of the machine, and in the case of the latter in the form of skin float and suspended agglomerates at the table side. Such devices may be used in practicing the improved method of the present invention.

In the commercial practice of the process of the Crago patent it sometimes occurs that, while the final phosphate concentrate produced is of high grade, the percentage of the available phosphate in the feed which appears in the final phosphate concentrate is not as high as desired. That is, although a phosphate concentrate of high grade is obtained, a considerable percentage of the phosphate in the feed has been collected with the siliceous gangue and sent to waste in the last step of the process.

Difficulty in obtaining recovery in the final phosphate concentrate of a satisfactory percentage of the phosphate in the feed, as above mentioned, seems to be due to a number of causes which are more likely to occur in plant operation than in laboratory practicing of the method of said Crago patent. My belief is that when the unsatisfactory percentage of recovery just mentioned is encountered it is due to failure adequately to treat the rougher concentrate with a mineral acid to remove the effect of the reagents used in its production. In a plant operation, that failure may be due to the use of insufficient mineral acid or to lack of adequate mixing of the acid with the rougher concentrate or to both, or to other reasons. Various attempts have been made to insure a high percentage of phosphate recovery in practicing the method of the Crago patent, but these attempts have either been more or less unsuccessful or have required the use of additional reagents or apparatus or both, which has increased the cost and complexity of the plant and its operation.

The general object of the present invention is to make more certain a high percentage recovery of phosphate in the final phosphate concentrate

produced by the method of said Crago patent. According to the present invention, the desired end is achieved, with economy in the use of reagents and without substantial increase in the apparatus employed in the plant, by subjecting the acid-treated rougher phosphate concentrate to treatment resulting in the removal therefrom of a high-grade concentrate of the phosphate values; whereupon the residue of that treatment is subjected in an aqueous pulp to a concentrating operation (according to the last step of the method of the Crago patent) to remove a collected material largely composed of siliceous gangue which is sent to waste; after which the residue from the last mentioned operation and the phosphate concentrate resulting from the first mentioned operation are combined to produce the final high-grade concentrate containing a high proportion of the phosphate in the ore. In practicing the improved process, I have discovered that, prior to subjecting the acid-treated rougher phosphate concentrate to treatment to remove therefrom a phosphate concentrate, treatment with an inert oil such as kerosene or pine oil or both is advantageous. While kerosene seems to be preferable as the inert oil, other hydrocarbon oils such as light gravity petroleum oils may be employed. When pine oil is used, it acts both as a frothing agent and as an inert oil in the treatment. The amount of the phosphate concentrate obtained by this concentrating operation, following the acid treatment of the rougher phosphate concentrate, is of course relatively small, but this concentrate is of high grade; and the removal of this phosphate concentrate from the material that is the feed to the last step of the method of the Crago patent, substantially prevents phosphate from being separated from that feed along with the siliceous gangue which is sent to waste.

An important advantage of the present invention is that it requires the use of only small amounts of reagents and calls for very little additional plant equipment. For example, in plants where the final operation of the method of the Crago patent had been performed in a bank of flotation cells, the inert oil or oils may be introduced into the feed to the first of those cells, and the froth-floated phosphate concentrate from that cell may be removed; the positive-ion reagents are introduced into the machine discharge from that first cell which is fed to the remaining cells from which froth-floated siliceous gangue is removed and sent to waste; after which the froth-floated phosphate concentrate from the first cell and the machine discharge of the other cells are combined to form the final phosphate concentrate.

The method of the present invention will be understood from the following description, taken in connection with the accompanying drawing which shows a flow-sheet of a typical plant practicing the method. It will be understood that this flow-sheet is merely an aid to the understanding of the invention, and that various modifications in the apparatus referred to in the flow-sheet may be resorted to without departing from the spirit of the invention as defined in the claims hereto appended.

Referring to the flow-sheet shown in the drawing, it will be evident that the four steps of the improved method are separated by dash lines. The first step results in obtaining, from the raw phosphate feed to the plant, of a rougher phosphate concentrate; the second step involves the

acid-treating of that rougher phosphate concentrate thereby obtaining an acid-treated rougher phosphate concentrate, according to the teachings of the said Crago patent; the third (new) step involves the treating of said acid-treated rougher phosphate concentrate with inert oils and the removal of a phosphate concentrate which is a part of the final phosphate concentrate; and the fourth step involves the treating of the machine discharge from the third step with a positive-ion reagent, followed by flotation treatment which eliminates a siliceous froth product which is sent to waste; leaving the machine discharge as a phosphate concentrate which is combined with the phosphate concentrate produced in the third step, to give the final phosphate concentrate.

The invention and the advantages thereof will be understood from consideration of tests which will now be described. Test 1 shows the results from use of the invention, when the acid-treating of the rougher phosphate concentrate in the second step of the method is inadequate to remove the effect of the reagents used in the production of the rougher phosphate concentrate. Test 2 shows the results when, in practicing the invention, the acid-treating of the rougher phosphate concentrate in the second step is more nearly adequate to remove the effect of the reagents used in the production of the rougher phosphate concentrate. Test 3 shows the results of practicing the invention, when the acid treatment of the second step is still more nearly adequate to remove the effect of the reagents used in the production of the rougher phosphate concentrate. In carrying out these tests, the adequacy of the acid treating step was increased from Test No. 1 to Test No. 2 to Test No. 3, by increasing the amount of mineral acid used; but it is to be understood that in plant operation the adequacy of the acid-treating step may depend on other factors than the amount of acid used, for example, the thoroughness with which the acid is mixed with the rougher phosphate concentrate in the acid agitator, and by other factors. For the purpose of explaining and demonstrating the advantages of the present invention, varying the amount of mineral acid employed to remove the effect of the reagents used in the production of the rougher phosphate concentrate is a simple method for varying the adequacy of the acid treatment of the rougher phosphate concentrate.

In each of the three tests hereinafter described, the feed was obtained from deslimed, minus 14-mesh, phosphate ore which was screened on a 35-mesh screen so as to obtain the minus 35-mesh fraction of the ore which was used as the feed. In each of the tests, this feed, which contained about 35.7% B. P. L. (bone phosphate of lime), was conditioned at about 70% solids with 0.5 lb. caustic soda, 4.4 lbs. fuel oil and 1.1 lbs. tall oil fatty acid, per ton of solids, for about two minutes. Then this conditioned feed was subjected to froth-flotation treatment resulting in the production in a froth-float of a rougher phosphate concentrate, the siliceous machine discharge being sent to waste. The rougher phosphate concentrate so obtained was dewatered to approximately 50% solids and then agitated for about two minutes with sulfuric acid, after which the solids were washed substantially free from slimes, reagents and acid; the amount of sulfuric acid used being 1.0 lb., 2.0 lbs. and 4.0 lbs. in Tests Nos. 1, 2 and 3, respectively. The washed, acid-treated, rougher

phosphate concentrate thus obtained was then made into a thin pulp at about 10% solids, and fed to a froth-flotation cell in which it was conditioned for about 15 seconds with 1.8 lbs. kerosene and 0.1 lb. pine oil, per ton of solids, after which a froth-float in the form of a phosphate concentrate was removed. The machine discharge from the last mentioned operation was then fed to a froth-flotation cell in which it was conditioned for about 15 seconds with 0.2 lb. octadecylamine acetate, per ton of solids, and the resulting silicious froth-float was sent to waste, leaving the machine discharge as a phosphate concentrate which was combined with the phosphate concentrate resulting from the previous step, thereby producing a final phosphate concentrate of high grade with a recovery of a high percentage of the phosphate in the original feed. It will be noted that the conditions in Tests 1, 2 and 3 were the same, except that the amount of sulfuric acid employed was 1.0 lb., 2.0 lbs. and 4.0 lbs. in the respective tests. The interesting metallurgical results of Tests 1, 2 and 3 are shown in the following tables:

TABLE 1

Phosphate concentrate (froth product) obtained after treatment with inert oils—3rd step

| Test   | Wt.      | B. P. L. | Ins.     | B. P. L.<br>Rec. |
|--------|----------|----------|----------|------------------|
|        | Per cent | Per cent | Per cent | Per cent         |
| 1..... | 15.5     | 76.3     | 4.8      | 32.9             |
| 2..... | 1.2      | 75.8     | 4.0      | 2.5              |
| 3..... | 0.2      | 72.1     | 9.3      | 0.3              |

TABLE 2

Phosphate concentrate (machine discharge) obtained after treatment with positive-ion reagents—4th step

| Test   | Wt.      | B. P. L. | Ins.     | B. P. L.<br>Rec. |
|--------|----------|----------|----------|------------------|
|        | Per cent | Per cent | Per cent | Per cent         |
| 1..... | 27.5     | 79.0     | 1.8      | 60.4             |
| 2..... | 41.6     | 78.8     | 1.9      | 92.1             |
| 3..... | 42.2     | 80.0     | 1.5      | 93.9             |

TABLE 3

Final phosphate concentrate—combined concentrates obtained by 3rd and 4th steps

| Test   | Wt.      | B. P. L. | Ins.     | B. P. L.<br>Rec. |
|--------|----------|----------|----------|------------------|
|        | Per cent | Per cent | Per cent | Per cent         |
| 1..... | 43.0     | 77.9     | 2.8      | 93.3             |
| 2..... | 42.8     | 78.7     | 2.1      | 94.6             |
| 3..... | 42.4     | 80.0     | 1.5      | 94.2             |

From consideration of the foregoing tables, it will be evident that each of the three tests produced a final phosphate concentrate of high grade (% B. P. L.) with high recovery (% B. P. L. Rec.), in spite of the wide differences in the adequacy of the treatment with acid to remove the effect of the reagents used in the production of the rougher phosphate concentrate.

Test 1 illustrates the usefulness of the invention when the effects of the reagents used in obtaining the rougher phosphate concentrate have been far from eliminated by the use of only 1.0 lb. sulfuric acid. As shown in Table 1, the phosphate concentrate (froth product) obtained after treatment with inert oils, was 15.5%

of the weight of the original feed, and had a grade of 76.3% B. P. L. with B. P. L. recovery of 32.9%. As shown in Table 2, the phosphate concentrate (machine discharge) obtained after treatment with positive-ion reagents, was 27.5% of the weight of the original feed, and had a grade of 79.0% B. P. L. with a B. P. L. recovery of only 60.4%. Nevertheless, as shown in Table 3, the final phosphate concentrate was 43.0% of the weight of the original feed, and had a grade of 77.9% B. P. L. with B. P. L. recovery of 93.3%.

Test 2 illustrates the usefulness of the invention when the effects of the reagents used in obtaining the rougher concentrate have been largely eliminated, as would be customary in a plant practicing the invention, by the use of 2.0 lbs. sulfuric acid. In this case, as shown in Table 1, the phosphate concentrate (froth product) obtained after treatment with inert oils had a grade of 75.8% B. P. L. (nearly as high as the corresponding grade in Test 1), but was only 1.2% of the weight of the original feed, with B. P. L. recovery of only 2.5%. Also, it will be noted that in Test 2, as shown in Table 2, the phosphate concentrate (machine discharge) obtained after treatment with positive-ion agents, was 41.6% of the weight of the original feed with 92.1% B. P. L. recovery, both of which results were far better than in Test 1. Moreover, as will be evident from Table 3, the final phosphate concentrate obtained by Test 2 had somewhat better metallurgical characteristics than in Test 1. Test 2 may be regarded as a good example of the practice of the method of the present invention, with economy in the use of reagents.

Test 3 is included merely for the purpose of demonstrating the correctness of the theories advanced in this specification, including the observation that in practicing the method of the Crago patent, failure to obtain high B. P. L. recovery is due to not sufficiently eliminating the effects of the reagents used in obtaining the rougher concentrate. In this test, the extravagant use of 4.0 lbs. sulfuric acid evidently almost completely eliminated those effects. Under these circumstances, it will be noted from Table 1 that the phosphate concentrate (froth product) obtained after treatment with inert oils was so insignificant in weight and so low in B. P. L. recovery that in this case the third step of the method had but little effect upon the final phosphate concentrate described in Table 3.

Thus, the results of Tests 1, 2 and 3 prove the usefulness in plant operation of the third step in the method of this invention. That is, the present method insures the obtaining of a highly satisfactory final concentrate, from the standpoints of weight, grade and recovery, in spite of wide variations in the adequacy of the acid treatment intended to remove the effects of the reagents used in the production of the rougher phosphate concentrate. Thus the method of the present invention generally gives more uniformly satisfactory and economical results in plant operation, than does the method of the Crago patent hereinbefore mentioned.

In practicing the method of the Crago patent, it is customary in some cases to subject the rougher phosphate concentrate produced by the first step to a cleaning operation before subjecting it to the acid treatment. In the tests hereinbefore described, this cleaning operation was not used, but of course it is to be understood that such a cleaning operation may be used in the present method without departing from the spirit

of the invention, and that in the following claims the expression "rouger concentrate of the phosphate values mixed with silicious gangue" is intended to refer to the product resulting from the first step of the method, whether or not that product is subjected to a cleaning operation prior to the acid treatment of it.

What is claimed is:

1. A method of concentrating phosphate minerals from their ores, which comprises subjecting the ore in an aqueous pulp to a concentrating operation with negative-ion reagents to separate a rougher floating concentrate of the phosphate values mixed with silicious gangue, conditioning an aqueous pulp of that rougher phosphate concentrate with a mineral acid and then dewatering said pulp thereby eliminating a large part of said mineral acid and also the agents used in the production of that rougher phosphate concentrate, adding an inert oil to an aqueous pulp of that acid-treated rougher phosphate concentrate and subjecting said pulp to a concentrating operation resulting in the removal and saving of a high-grade floating concentrate of a part of the phosphate values, subjecting the residue of that operation in an aqueous pulp to a concentrating operation with added positive-ion reagents to remove and discard a floated material largely composed of silicious gangue, and combining the residue from that operation with the previously mentioned high-grade phosphate concentrate, thereby producing a final high-grade phosphate concentrate containing a high proportion of the phosphate in the ore.

2. A method of concentrating phosphate minerals from their ores, which comprises subjecting the ore in an aqueous pulp to a concentrating operation with negative-ion reagents to separate a rougher floating concentrate of the phosphate values mixed with silicious gangue, conditioning an aqueous pulp of that rougher phosphate concentrate with a mineral acid and then dewatering

- 5 said pulp and washing it with water thereby eliminating substantially all of said mineral acid and the agents used in the production of that rougher phosphate concentrate, adding an inert oil to an aqueous pulp of that acid-treated and washed rougher phosphate concentrate and subjecting it to a concentrating operation resulting in the removal and saving of a high-grade floating concentrate of a part of the phosphate values, subjecting the residue of that operation in an aqueous pulp to a concentrating operation with added positive-ion reagents to remove and discard a floated material largely composed of silicious gangue, and combining the residue from that operation with the previously mentioned high-grade phosphate concentrate, thereby producing a final high-grade phosphate concentrate containing a high proportion of the phosphate in the ore.
- 10 20 3. A method according to claim 1, in which the inert oil is a mineral oil.
4. A method according to claim 1, in which the inert oil is a frothing agent.
- 15 25 5. A method according to claim 1, in which the inert oil is kerosene.
6. A method according to claim 1, in which the inert oil is pine oil.
- 20 30 7. A method according to claim 1, in which the inert oil is a mixture of kerosene and pine oil.

JAMES B. DUKE.

#### REFERENCES CITED

The following references are of record in the file of this patent:

#### UNITED STATES PATENTS

| Number    | Name       | Date          |
|-----------|------------|---------------|
| 2,175,724 | Gaudin     | Apr. 2, 1940  |
| 2,293,840 | Crago      | Aug. 18, 1942 |
| 2,389,727 | Herkenhoff | Nov. 27, 1945 |